



US011104860B2

(12) **United States Patent**  
**Chen et al.**

(10) **Patent No.:** **US 11,104,860 B2**  
(b4) **Date of Patent:** **Aug. 31, 2021**

(54) **LUBRICATING OILS**(71) Applicant: **CRODA, INC.**, Edison, NJ (US)(72) Inventors: **Xin Chen**, Hockessin, DE (US); **Alexei Nikolaeovich Kurchan**, Wallingford, PA (US); **Zhongqi Shen**, Plainsboro, NJ (US)(73) Assignee: **Croda, Inc.**, Plainsboro, NJ (US)

(\* ) Notice: Subject to any disclaimer, the term of this patent is extended or adjusted under 35 U.S.C. 154(b) by 0 days.

(21) Appl. No.: **15/310,988**(22) PCT Filed: **May 14, 2015**(86) PCT No.: **PCT/US2015/030771**

§ 371 (c)(1),

(2) Date: **Nov. 14, 2016**(87) PCT Pub. No.: **WO2015/175778**PCT Pub. Date: **Nov. 19, 2015**(65) **Prior Publication Data**

US 2017/0073609 A1 Mar. 16, 2017

**Related U.S. Application Data**

(60) Provisional application No. 61/993,520, filed on May 15, 2014.

(51) **Int. Cl.****C10M 163/00** (2006.01)**C10M 169/04** (2006.01)**C10M 133/16** (2006.01)**C10M 133/18** (2006.01)**C10M 105/68** (2006.01)**C10M 135/18** (2006.01)**C10N 20/02** (2006.01)**C10N 20/00** (2006.01)**C10N 30/00** (2006.01)**C10N 40/04** (2006.01)**C10N 40/08** (2006.01)**C10N 40/20** (2006.01)**C10N 40/22** (2006.01)**C10N 40/24** (2006.01)**C10N 40/25** (2006.01)**C10N 40/30** (2006.01)(52) **U.S. Cl.**CPC ..... **C10M 169/04** (2013.01); **C10M 105/68** (2013.01); **C10M 133/16** (2013.01); **C10M 133/18** (2013.01); **C10M 135/18** (2013.01); **C10M 2203/024** (2013.01); **C10M 2205/0285** (2013.01); **C10M 2207/289** (2013.01); **C10M 2215/08** (2013.01); **C10M 2215/10** (2013.01); **C10M 2219/068** (2013.01); **C10N 2020/02** (2013.01); **C10N 2020/083** (2020.05); **C10N 2020/085** (2020.05); **C10N 2030/66** (2020.05); **C10N 2030/70** (2020.05); **C10N 2030/74** (2020.05); **C10N 2040/04** (2013.01); **C10N**2040/08 (2013.01); **C10N 2040/20** (2013.01); **C10N 2040/22** (2013.01); **C10N 2040/24** (2013.01); **C10N 2040/25** (2013.01); **C10N 2040/30** (2013.01)(58) **Field of Classification Search**CPC ..... C10M 133/16; C10M 2215/12  
USPC ..... 508/364, 528  
See application file for complete search history.(56) **References Cited**

## U.S. PATENT DOCUMENTS

|               |         |                   |
|---------------|---------|-------------------|
| 2,686,811 A   | 8/1954  | Bull              |
| 3,278,612 A   | 10/1966 | Greene            |
| 3,312,620 A * | 4/1967  | Low .....         |
|               |         | C10M 3/00         |
|               |         | 508/254           |
| 3,827,981 A   | 8/1974  | Thompson          |
| 3,894,958 A * | 7/1975  | McCoy .....       |
|               |         | C10M 169/00       |
|               |         | 508/469           |
| 3,910,847 A   | 10/1975 | Thompson          |
| 3,915,876 A   | 10/1975 | Thompson          |
| 3,953,346 A * | 4/1976  | Thompson .....    |
|               |         | C09K 5/08         |
|               |         | 508/555           |
| 4,096,077 A   | 6/1978  | Swakon            |
| 4,207,263 A   | 6/1980  | Hoffmann et al.   |
| 4,289,636 A   | 9/1981  | Davis et al.      |
| 4,425,248 A   | 1/1984  | Piotrowski et al. |
| 4,579,673 A   | 4/1986  | Piotrowski et al. |
| 4,992,188 A   | 2/1991  | Jolley            |

(Continued)

## FOREIGN PATENT DOCUMENTS

|    |              |        |
|----|--------------|--------|
| DE | 202009016945 | 3/2010 |
| EP | 0188786      | 7/1986 |

(Continued)

## OTHER PUBLICATIONS

International Search Report for PCT/US2015/030771, dated Oct. 8, 2015, 3 pages.

(Continued)

Primary Examiner — Prem C Singh

Assistant Examiner — Francis C Campanell

(74) Attorney, Agent, or Firm — RatnerPrestia

(57) **ABSTRACT**

A lubricating composition comprises an amide and at least one additive. The amide is the reaction product of a secondary, branched amine and a carboxylic acid. The carboxylic acid may be a monocarboxylic acid or a dicarboxylic acid, including dimer acid. The amide is hydrolytically stable, and may be used to increase the hydrolytic stability of the lubricant composition. Alternatively, the amide may be used to increase the additive solubility or detergency of the lubricant composition.

(56)

**References Cited**

U.S. PATENT DOCUMENTS

|                   |         |                |             |
|-------------------|---------|----------------|-------------|
| 5,194,171 A *     | 3/1993  | Jolley .....   | C10M 105/68 |
|                   |         |                | 252/67      |
| 9,562,207 B2      | 2/2017  | DeBlase et al. |             |
| 2007/0027044 A1 * | 2/2007  | Le Coent ..... | C07G 17/008 |
|                   |         |                | 508/460     |
| 2007/0232833 A1   | 10/2007 | Haese et al.   |             |
| 2009/0131293 A1 * | 5/2009  | Ma .....       | C08K 5/18   |
|                   |         |                | 508/563     |

FOREIGN PATENT DOCUMENTS

|    |                 |        |
|----|-----------------|--------|
| EP | 1876285         | 1/2008 |
| JP | 4970917 A       | 7/1974 |
| JP | 524968 A        | 1/1977 |
| JP | S52004968 A     | 1/1977 |
| KR | 1020080086401 A | 9/2008 |

OTHER PUBLICATIONS

International Preliminary Report on Patentability and Written Opinion for International Application No. PCT/US2015/030771, dated Nov. 15, 2016, 8 pages.

Chinese Office Action for Chinese Application No. 201580025931. X, dated Oct. 24, 2018, with translation, 21 pages.

Notice of Reasons for Rejection for Japanese Application No. 2016-667692, dated Jan. 16, 2019 with translation, 6 pages.

Korean Notification of Reasons for Refusal for Korean Application No. 10-2016-7034739, dated May 26, 2020 with translation, 15 pages.

\* cited by examiner

# 1

## LUBRICATING OILS

### CROSS REFERENCE TO RELATED APPLICATION

This application claims priority to U.S. Provisional Application No. 61/993,520, filed May 15, 2014, the entire disclosure of which is incorporated herein by reference in its entirety for all purposes.

### FIELD OF THE INVENTION

The present invention relates to a lubricant composition. The lubricant composition may be used in the automotive, marine, industrial, compressor, refrigeration or other lubrication fields. In particular, the present invention relates to a lubricant composition comprising an amide, more preferably an oil-soluble amide, as the base fluid or an additive.

### BACKGROUND

Lubricant compositions typically comprise a lubricant base stock and an additive package, both of which can contribute significantly to the properties and performance of the lubricant composition.

The choice of lubricant base stock can have a major impact on properties such as oxidation and thermal stability, volatility, low temperature fluidity, solvency of additives, contaminants and degradation products, and traction. The American Petroleum Institute (API) currently defines five groups of lubricant base stocks (API Publication 1509) for automotive engine oils.

Groups I, II and III are mineral oils which are classified by the amount of saturates and sulphur they contain and by their viscosity indices. Table 1 below illustrates these API classifications for Groups I, II and III.

TABLE 1

| Group | Saturates    | Sulphur             | Viscosity Index (VI) |
|-------|--------------|---------------------|----------------------|
| I     | <90%         | >0.03%              | 80-120               |
| II    | At least 90% | Not more than 0.03% | 80-120               |
| III   | At least 90% | Not more than 0.03% | At least 120         |

Group I base stocks are solvent refined mineral oils, which are the least expensive base stock to produce, and currently account for the majority of base stock sales. They provide satisfactory oxidation stability, volatility, low temperature performance and traction properties and have very good solvency for additives and contaminants. Group II base stocks are mostly hydroprocessed mineral oils, which typically provide improved volatility and oxidation stability as compared to Group I base stocks. The use of Group II stocks has grown to about 30% of the US market. Group III base stocks are severely hydroprocessed mineral oils or they can be produced via wax or paraffin isomerisation.

They are known to have better oxidation stability and volatility than Group I and II base stocks but have a limited range of commercially available viscosities.

Group IV base stocks differ from Groups I to III in that they are synthetic base stocks e.g. polyalphaolefins (PAOs). PAOs have good oxidative stability, volatility and low pour points. Disadvantages include moderate solubility of polar additives, for example antiwear additives.

Group V base stocks are all base stocks that are not included in Groups I to IV. Examples include alkyl naphthalenes, alkyl aromatics, vegetable oils, esters (including

polyol esters, diesters and monoesters), polycarbonates, silicone oils and polyalkylene glycols.

To create a suitable lubricant composition, additives are blended into the chosen base stock. The additives either enhance the stability of the lubricant base stock or provide additional functionalities to the composition. Examples of automotive engine oil additives include antioxidants, anti-wear agents, detergents, dispersants, viscosity index improvers, defoamers, pour point depressants and friction reducing additives.

Many lubricant base stocks and additives are based on esters; including monoesters, diesters and polyol esters. These ester compounds provide good properties, for example kinematic viscosities and viscosity indices, for lubricant compositions. However, the presence and nature of the ester group (—COO—) in these compounds leads to hydrolysis in systems where water may be present, and/or oxidation or thermal degradation in systems which are subjected to high temperatures.

There exists, therefore, a need for a lubricant composition which exhibits good hydrolytic stability, as well as possessing favourable physical properties for use in lubrication applications.

### SUMMARY OF THE INVENTION

It is an object of the present invention to address the above and/or other disadvantages associated with the prior art.

Thus, according to a first aspect of the present invention, there is provided a lubricating composition comprising:

- a) an amide which is the reaction product of a secondary, branched amine and a carboxylic acid; and
- b) at least one additive.

According to a second aspect of the present invention, there is provided a method of increasing the additive solubility or detergency of a lubricant composition which comprises using a lubricant composition comprising:

- a) an amide which is the reaction product of a secondary, branched amine and a carboxylic acid; and
- b) at least one additive.

In a preferred aspect, there is provided a method of increasing the additive solubility of a lubricant composition which comprises using a lubricant composition comprising:

- a) an amide which is the reaction product of a secondary, branched amine and a carboxylic acid; and
- b) at least one additive.

By the use of the term "additive solubility" as used herein, it is meant the ability of the additive or additives to dissolve within the lubricant composition to produce a clear, i.e. non-hazy, non-separated and sediment free, solution.

According to a third aspect of the present invention, there is provided the use of an amide which is the reaction product of a secondary, branched amine and a carboxylic acid to increase the additive solubility or detergency of a lubricant composition.

According to a further aspect of the present invention, there is provided the use of an amide which is the reaction product of a secondary, branched amine and a carboxylic acid to produce a hydrolytically stable lubricant composition.

The lubricant composition described herein can be used as an automotive or marine engine oil, an automotive or marine gear or transmission oil, an industrial gear oil or turbine oil, a hydraulic oil, a compressor oil, a cutting oil, a rolling oil, a drilling oil, a refrigeration oil and the like.

## DETAILED DESCRIPTION OF THE INVENTION

The amide which is the reaction product of the secondary, branched amide and the carboxylic acid is a tertiary amide. Preferably, the amide is sterically hindered. By the term "sterically hindered", it is meant that the amide group, —NCO—, is bonded to large and/or branched moieties which shield the amide group from further reaction. A "large" group can be taken to mean any branched or linear hydrocarbyl chain.

Preferably, the lubricant composition comprises an amide of Formula (Ia) or (Ib):



wherein:

R<sup>1</sup> and R<sup>2</sup> are independently selected from the group consisting of C<sub>3</sub> to C<sub>18</sub> linear or branched, saturated or unsaturated, hydrocarbyl groups;

R<sup>3</sup> is selected from the group consisting of C<sub>3</sub> to C<sub>50</sub> linear or branched, saturated or unsaturated hydrocarbyl groups;

R<sup>4</sup> is selected from the group consisting of C<sub>1</sub> to C<sub>50</sub> linear or branched, saturated or unsaturated hydrocarbylene groups; and

n is 0 or 1,

wherein at least one of R<sup>1</sup> and R<sup>2</sup> is branched.

By the term "hydrocarbyl group" as used herein, it is meant an acyclic or cyclic functional group consisting only of carbon and hydrogen atoms which is the fragment, containing an open point of attachment on a carbon atom, that would form if a hydrogen atom bonded to a carbon atom is removed from the molecule of a hydrocarbon. The definition of the term "hydrocarbyl group" when used herein includes alkyl (saturated), alkenyl (containing a carbon-carbon double bond) and alkynyl (containing a carbon-carbon triple bond) groups. Preferably, the hydrocarbyl groups referred to herein are alkyl or alkenyl groups, more preferably alkyl groups. Preferably, the hydrocarbyl groups referred to herein are acyclic.

By the term "hydrocarbylene group" as used herein, it is meant an acyclic or cyclic functional group consisting only of carbon and hydrogen atoms which is the fragment, containing two open points of attachment on a carbon atom, or one open point of attachment each on two separate carbon atoms, that would form if two hydrogen atoms were removed from the molecule of a hydrocarbon. The definition of the term "hydrocarbylene group" when used herein includes alkylene (saturated), alkenylene (containing a carbon-carbon double bond) and alkynylene groups (containing a carbon-carbon triple bond). Preferably, the hydrocarbylene groups referred to herein are alkylene or alkenylene groups, more preferably alkylene groups. Preferably, the hydrocarbylene groups referred to herein are acyclic. Preferably, the

open points of attachment on the hydrocarbylene groups are on the terminal carbon atoms of the hydrocarbylene chain.

The groups R<sup>1</sup> and R<sup>2</sup> are both present in the secondary, branched amine reactant. The groups R<sup>3</sup> and R<sup>4</sup>, when present, are present in the carboxylic acid reactant.

Preferably, R<sup>1</sup> and R<sup>2</sup> are independently of each other C<sub>3</sub> to C<sub>15</sub> hydrocarbyl groups, more preferably C<sub>3</sub> to C<sub>13</sub> hydrocarbyl groups, and most preferably C<sub>3</sub> to C<sub>10</sub> hydrocarbyl groups. Preferably, R<sup>1</sup> and R<sup>2</sup> are independently of each other C<sub>3</sub> to C<sub>15</sub> alkyl groups, more preferably C<sub>3</sub> to C<sub>13</sub> alkyl groups, and most preferably C<sub>3</sub> to C<sub>10</sub> alkyl groups.

Preferably both R<sup>1</sup> and R<sup>2</sup> are branched. Preferably, both R<sup>1</sup> and R<sup>2</sup> are saturated.

R<sup>1</sup> and R<sup>2</sup> may be the same or different. Preferably, R<sup>1</sup> and R<sup>2</sup> are the same as each other. Preferably, both R<sup>1</sup> and R<sup>2</sup> are branched, saturated, C<sub>3</sub> to C<sub>15</sub> alkyl groups, more preferably C<sub>3</sub> to C<sub>13</sub> alkyl groups, most preferably C<sub>3</sub> to C<sub>8</sub> alkyl groups.

R<sup>3</sup> is preferably a C<sub>2</sub> to C<sub>35</sub> hydrocarbyl group, preferably a C<sub>3</sub> to C<sub>23</sub> hydrocarbyl group, more preferably a C<sub>5</sub> to C<sub>21</sub> hydrocarbyl group and most preferably a C<sub>6</sub> to C<sub>17</sub> hydrocarbyl group. R<sup>3</sup> is preferably a C<sub>2</sub> to C<sub>35</sub> alkyl or alkenyl group, preferably a C<sub>3</sub> to C<sub>23</sub> alkyl or alkenyl group, more preferably a C<sub>5</sub> to C<sub>21</sub> alkyl or alkenyl group and most preferably a C<sub>6</sub> to C<sub>17</sub> alkyl or alkenyl group. R<sup>3</sup> is preferably a C<sub>2</sub> to C<sub>35</sub> alkyl group, preferably a C<sub>3</sub> to C<sub>23</sub> alkyl group, more preferably a C<sub>5</sub> to C<sub>21</sub> alkyl group and most preferably a C<sub>6</sub> to C<sub>17</sub> alkyl group.

Preferably, R<sup>4</sup> is a C<sub>1</sub> to C<sub>40</sub> hydrocarbylene group, preferably a C<sub>1</sub> to C<sub>16</sub> or a C<sub>24</sub> to C<sub>40</sub> hydrocarbylene group, more preferably a C<sub>1</sub> to C<sub>12</sub> or a C<sub>28</sub> to C<sub>38</sub> hydrocarbylene group and most preferably a C<sub>1</sub> to C<sub>8</sub> or a C<sub>34</sub> hydrocarbylene group. R<sup>4</sup> is preferably a C<sub>1</sub> to C<sub>40</sub> alkylene or alkenylene group, preferably a C<sub>1</sub> to C<sub>16</sub> or a C<sub>24</sub> to C<sub>40</sub> alkylene or alkenylene group, more preferably a C<sub>1</sub> to C<sub>12</sub> or a C<sub>28</sub> to C<sub>38</sub> alkylene or alkenylene group and most preferably a C<sub>1</sub> to C<sub>8</sub> or a C<sub>34</sub> alkylene or alkenylene group. R<sup>4</sup> is preferably an alkylene group.

Preferably, n is 1.

Preferably, the secondary, branched amine reactant has the formula (II):



wherein R<sup>1</sup> and R<sup>2</sup> are as defined above, and wherein at least one of R<sup>1</sup> and R<sup>2</sup> is branched. Preferably, both R<sup>1</sup> and R<sup>2</sup> are both branched. More preferably, R<sup>1</sup> and R<sup>2</sup> are the same as each other.

Examples of suitable secondary, branched amine reactants include, but are not limited to, di-(2-ethylhexyl)amine (alternative names: (Di-2-EHA) or Bis-(2-ethylhexyl)amine), available from OXEA and BASF), diisopropylamine (alternative names: N,N-Diisopropylamine or DIPA, produced as described in U.S. Pat. No. 2,686,811), ditridecylamine (mixture of isomers) (available from BASF), and diisobutylamine (alternative names: Bis(2-methylpropyl)amine, Di-isobutylamine or N,N-Bis(2-methylpropyl)amine, available from BASF, Shanghai Hanhong Chemical Co., Ltd. and others), more preferably di-(2-ethylhexyl)amine or diisopropylamine.

Secondary amines suitable for use in the present invention are generally produced from corresponding alcohols,

ketones or aldehydes and ammonia or primary amines, as described in following patents: U.S. Patent Application Publication No. 2007/0232833A1, U.S. Pat. No. 8,034,978B2, U.S. Pat. No. 4,207,263. Alcohols are often obtained via catalytic hydroformylation or hydrogenation (alternatively called the 'oxo-process') from corresponding olefins reacted with gas containing carbon monoxide, hydrogen and carbon dioxide (examples of processes are described in U.S. Pat. Nos. 3,278,612 A and 4,207,263).

The carboxylic acid reactant may be a monocarboxylic acid or a dicarboxylic acid. When the carboxylic acid is a monocarboxylic acid, the amide is preferably a monoamide. When the carboxylic acid is a dicarboxylic acid, the amide is preferably a diamide.

When the carboxylic acid is a monocarboxylic acid, the resulting amide is a compound of Formula (Ia).

In this embodiment, the monocarboxylic acid may be branched or linear and may be saturated or unsaturated. The monocarboxylic acid preferably comprises up to 36 carbon atoms, preferably up to 22 carbon atoms and most preferably up to 18 carbon atoms. The monocarboxylic acid preferably comprises at least 4 carbon atoms, preferably at least 6 carbon atoms and most preferably at least 8 carbon atoms. Examples of suitable branched and linear monocarboxylic acids include, but are not limited to linear acids such as hexanoic acid, heptanoic acid, caprylic acid, nonanoic acid, capric acid, lauric acid, myristic acid, palmitic acid, heptadecanoic acid, stearic acid, arachidic acid and behenic acid; iso-acids such as isostearic acid, isomyristic acid, isopalmitic acid, isopalmitic acid and isobehenic acid; neo-acids such as neocapric acid; anti-iso acids; polybranched acids such as 2-ethyl hexanoic acid and 3,5,5'-trimethylhexanoic acid; unsaturated acids such as oleic acid, iso-oleic acid, linoleic acid, linolenic acid, erucic acid and palmitoleic acid.

Preferably, the monocarboxylic acid is saturated. Preferably, the monocarboxylic acid is selected from the group comprising 2-ethyl hexanoic acid, 3,5,5'-trimethylhexanoic acid, caprylic/capric acid, lauric acid, stearic acid and isostearic acid. Preferably, the monocarboxylic acid is branched. Most preferably, the monocarboxylic acid is 2-ethyl hexanoic acid, 3,5,5'-trimethylhexanoic acid or isostearic acid.

When the carboxylic acid is a dicarboxylic acid, the resulting amide is a compound of Formula (Ib).

In one embodiment, the dicarboxylic acid is a linear or branched, saturated or unsaturated divalent C<sub>2</sub> to C<sub>14</sub> acid. In this embodiment, the dicarboxylic acid preferably comprises up to 12 carbon atoms and most preferably up to 10 carbon atoms. In this embodiment, the dicarboxylic acid may be selected from the group comprising oxalic acid, malonic acid, succinic acid, maleic acid, glutaric acid, adipic acid, pimelic acid, suberic acid, azelaic acid, sebatic acid, undecanoic acid and dodecanoic acid, preferably adipic acid, suberic acid and sebatic acid, more preferably adipic acid.

Preferably, the dicarboxylic acid is linear. Preferably, the dicarboxylic acid is saturated.

The dicarboxylic acid may be a dimer acid. In this embodiment, the dimer acid preferably comprises from 24 to 52 carbon atoms, preferably from 28 to 48 carbon atoms, more preferably from 32 to 46 carbon atoms and most preferably from 36 to 44 carbon atoms. Preferably the dimer acid is a C<sub>36</sub> dimer acid.

The term "dimer fatty acid" is well known in the art and refers to the dimerisation product of mono- or polyunsaturated fatty acids and/or esters thereof. Preferred dimer acids are dimers of C<sub>10</sub> to C<sub>30</sub>, more preferably C<sub>12</sub> to C<sub>24</sub>, particularly C<sub>14</sub> to C<sub>22</sub>, and especially C<sub>18</sub> alkyl chains.

Suitable dimer fatty acids include the dimerisation products of oleic acid, linoleic acid, linolenic acid, palmitoleic acid, and elaidic acid. The dimerisation products of the unsaturated fatty acid mixtures obtained in the hydrolysis of natural fats and oils, e.g. sunflower oil, soybean oil, olive oil, rapeseed oil, cottonseed oil and tall oil, may also be used. Hydrogenated, for example by using a nickel catalyst, dimer fatty acids may also be employed.

In addition to the dimer fatty acids, dimerisation usually results in varying amounts of oligomeric fatty acids (so-called "trimer") and residues of monomeric fatty acids (so-called "monomer"), or esters thereof, being present. The amount of monomer can, for example, be reduced by distillation. Particularly preferred dimer fatty acids have a dicarboxylic (or dimer) content of greater than 70%, more preferably greater than 85%, and particularly greater than 94% by weight.

The carboxylic acid is preferably a monocarboxylic acid.

Mixtures of said carboxylic acids could be used as the starting material for the production of the amide. Where mixtures of carboxylic acids are employed, preferably the mixtures are mixtures of two or more monocarboxylic acids or mixtures of two or more dicarboxylic acids, more preferably mixtures of two monocarboxylic acids. Said mixtures of acids may be commercially available as mixtures, for example capric and caprylic acids which are commercially available as C-810L™ from Proctor & Gamble.

Carboxylic acids suitable for use herein can be obtained from natural sources such as, for example plant or animal esters. For example, the acids may be obtained from palm oil, rape seed oil, palm kernel oil, coconut oil, babassu oil, soybean oil, castor oil, sunflower oil, olive oil, linseed oil, cottonseed oil, safflower oil, tallow, whale or fish oils, grease, lard and mixtures thereof. The carboxylic acids can also be synthetically prepared. Relatively pure unsaturated carboxylic acids such as oleic acid, linoleic acid, linolenic acid, palmitoleic acid, and elaidic acid may be isolated, or relatively crude unsaturated carboxylic acid mixtures employed. Resin acids, such as those present in tall oil, may also be used.

As will be appreciated, the acids and amines used to make said amides in the present invention will be from commercial sources and may not necessarily comprise 100 wt % of the acid or alcohol component under consideration. Such commercial products usually comprise a major proportion of the primary product together with other isomers and/or additional products of shorter or longer chain length. This may lead to variations in properties of the amides which are reaction products of the amidation reactions.

Preferably, the amide has a kinematic viscosity at 40° C., measured according to the method set out in ASTM D445, of at least 5 cSt, preferably at least 10 cSt, more preferably at least 15 cSt. Preferably, the amide has a kinematic viscosity at 40° C., measured according to the method set out in ASTM D445, of up to 320 cSt, preferably up to 280 cSt, more preferably up to 250 cSt.

Preferably, the amide has a kinematic viscosity at 100° C., measured according to the method set out in ASTM D445, of at least 1 cSt, preferably at least 2 cSt, more preferably at least 2.5 cSt. Preferably, the amide has a kinematic viscosity at 100° C., measured according to the method set out in ASTM D445, of up to 50 cSt, preferably up to 45 cSt, more preferably up to 40 cSt.

Preferably, the amide has a pour point, measured according to the method set out in ASTM D97, of not more than about -20° C., more particularly of not more than -25° C. and especially not more than -30° C.

Preferably, the neat amide has a hydrolytic stability measured according to the method set out in ASTM D943 of at least 40 hours, preferably at least 45 hours and most preferably at least 50 hours.

The lubricant composition may comprise one or more amide components. Preferably, the lubricant composition comprises only one amide component.

Where the lubricant composition comprises two or more amides, each amide may be selected with different properties. Preferably, the properties of each amide are within the values of such properties as described above. However, alternatively, one or more of the properties of at least one amide may be outside the values of such properties as described above provided that the properties of the mixture of amides are within the values of such properties as described above.

Preferably, the lubricant composition is non-aqueous. However, it will be appreciated that components of the lubricant composition may contain small amounts of residual water (moisture) which may therefore be present in the lubricant composition. The lubricant composition may comprise less than 5% water by weight based on the total weight of the composition. More preferably, the lubricant composition is substantially water free, i.e. contains less than 2%, less than 1%, or preferably less than 0.5% water by weight based on the total weight of the composition.

Preferably the lubricant composition is substantially anhydrous.

The lubricant composition may comprise at least 0.1 wt % of said at least one additive, preferably at least 0.5 wt %, more preferably at least 1 wt %, and desirably at least 2 wt % based on the total weight of the composition. The lubricant composition may comprise up to 40 wt % of said at least one additive, preferably up to 30 wt %, more preferably up to 20 wt % and desirably up to 10 wt % based on the total weight of the composition.

The lubricant composition may be an engine oil, hydraulic oil or fluid, gear oil, chain oil, metal working fluid or refrigerant oil. To adapt the lubricant composition to its intended use, the lubricant composition may comprise one or more of the following additive types.

1. Dispersants: for example, alkenyl succinimides, alkenyl succinate esters, alkenyl succinimides modified with other organic compounds, alkenyl succinimides modified by post-treatment with ethylene carbonate or boric acid, pentaerythritols, phenate-salicylates and their post-treated analogs, alkali metal or mixed alkali metal, alkaline earth metal borates, dispersions of hydrated alkali metal borates, dispersions of alkaline-earth metal borates, polyamide ashless dispersants and the like or mixtures of such dispersants.

2. Anti-oxidants: Anti-oxidants reduce the tendency of mineral oils to deteriorate in service which deterioration is evidenced by the products of oxidation such as sludge and varnish-like deposits on the metal surfaces and by an increase in viscosity. Examples of anti-oxidants include phenol type (phenolic) oxidation inhibitors, such as 4,4'-methylene-bis(2,6-di-tert-butylphenol), 4,4'-bis(2,6-di-tert-butylphenol), 4,4'-bis(2-methyl-6-tert-butylphenol), 2,2'-methylene-bis(4-methyl-6-tert-butyl-phenol), 4,4'-butylidene-bis(3-methyl-6-tert-butylphenol), 4,4'-isopropylidene-bis(2,6-di-tert-butylphenol), 2,2'-methylene-bis(4-methyl-6-nonylphenol), 2,2'-isobutylidene-bis(4,6-dimethylphenol), 2,2'-methylene-bis(4-methyl-6-cyclohexylphenol), 2,6-di-tert-butyl-4-methylphenol, 2,6-di-tert-butyl-4-ethylphenol, 2,6-di-tert-butylphenol, 2,4-dimethyl-6-tert-butyl-phenol, 2,6-di-tert-1-dimethylamino-p-cresol, 2,6-di-tert-4-(N,N'-dimethylamino-methylphenol),

4,4'-thiobis(2-methyl-6-tert-butylphenol), 2,2'-thiobis(4-methyl-6-tert-butylphenol), bis(3-methyl-4-hydroxy-5-tert-butylbenzyl)-sulfide, and bis(3,5-di-tert-butyl-4-hydroxybenzyl). Other types of oxidation inhibitors include alkylated diphenylamines (e.g., IRGANOX® L-57 from Ciba-Geigy), metal dithiocarbamate (e.g., zinc dithiocarbamate), and methylenebis(dibutylidithiocarbamate).

3. Antiwear agents: As their name implies, these agents reduce wear of moving metallic parts. Examples of such agents include phosphates, phosphites, carbamates, esters, sulfur containing compounds, and molybdenum complexes.

4. Emulsifiers: for example, linear alcohol ethoxylates.

5. Demulsifiers: for example, addition products of alkylphenol and ethylene oxide, polyoxyethylene alkyl ethers, and polyoxyethylene sorbitan esters.

6. Extreme pressure agents (EP agents): for example, zinc dialkylidithiophosphate (primary alkyl, secondary alkyl, and aryl type), sulfurized oils, diphenyl sulfide, methyl trichlorostearate, chlorinated naphthalene, fluoroalkylpolysiloxane, and lead naphthenate. A preferred EP agent is zinc dialkyl dithiophosphate (ZnDTP or ZDDP), e.g. as one of the co-additive components for an antiwear hydraulic fluid composition.

7. Multifunctional additives: for example, sulfurized oxy-molybdenum dithiocarbamate, sulfurized oxymolybdenum organo phosphorodithioate, oxymolybdenum monoglycchde, oxymolybdenum diethylate amide, amine-molybdenum complex compound, and sulfur-containing molybdenum complex compound.

8. Viscosity index improvers: for example, polymethacrylate polymers, ethylene-propylene copolymers, styrene-isoprene copolymers, hydrogenated styrene-isoprene copolymers, polyisobutylene, and dispersant type viscosity index improvers.

9. Pour point depressants: for example, polymethacrylate polymers.

10. Foam inhibitors: for example, alkyl methacrylate polymers and dimethyl silicone polymers.

11. Friction modifying agents, preferably friction reducing agents: for example, esters, partial esters, phosphonates, organomolybdenum-based compounds, fatty acids, higher alcohols, fatty acid esters, sulfur containing esters, phosphate esters, acid phosphoric acid esters, and amine salts of phosphoric acid esters.

12. The additive or additives may be available in the form of a commercially available additive pack. Such additive packs vary in composition depending on the required use of the additive pack. A skilled person may select a suitable commercially available additive pack for each of: an engine oil, a gear oil, a hydraulic fluid and a metal working fluid. An example of a suitable additive pack for an engine oil is HITEC® 11100 (ex. Afton Chemical Corporation, US) which is recommended to be used at about 10 wt % of the lubricant composition. An example of a suitable additive pack for a gear oil is ADDITIN® RC 9451 (ex. Rhein Chemie Rheinau GmbH, Germany) which is recommended to be used at between 1.5 to 3.5 wt % of the lubricant composition.

13. An example of a suitable additive pack for a hydraulic oil or fluid is ADDITIN® RC 9207 (ex. Rhein Chemie Rheinau GmbH, Germany) which is recommended to be used at about 0.85 wt % of the lubricant composition.

14. An example of a suitable additive pack for a metal working fluid is ADDITIN® RC 9410 (ex. Rhein Chemie Rheinau GmbH, Germany) which is recommended to be used at between 2 to 7 wt % of the lubricant composition.

15. The lubricant composition according to the present invention may comprise said amide and said at last one additive

along with a further base oil, or may consist essentially of said amide and said additive(s).

When the lubricant composition does not consist essentially of said amide and said additive(s), the balance of the lubricant composition comprises a further base oil which is a lubricant component selected from API Groups I, II, III, III+ (including gas-to-lubricants), IV, IV+ and V lubricants and mixtures of two or more thereof.

Examples of suitable Group III lubricants include mineral oils. Examples of suitable Group IV lubricants included poly- $\alpha$ -olefins derived from C<sub>8</sub> to C<sub>12</sub>  $\alpha$ -olefins and having kinematic viscosities in the range 3.6 cSt to 8 cSt at 100° C. Examples of Group V lubricants include alkyl naphthalenes, alkyl benzenes and esters, for example esters derived from monohydric alcohols and/or polyols and monocarboxylic acids or polycarboxylic acids. Examples of alkyl naphthalenes include SYNESSTIC™ 5 and SYNESSTIC™ 12 alkyl naphthalenes available from Mobil. Examples of esters are PRIOLUBE™ 1976 a monoester and PRIOLUBE™ 3970 a TMP nC<sub>8</sub>/nC<sub>10</sub> polyol ester. GTL base stocks are made by conversion of natural gas (i.e., methane and higher alkanes) to synthesis gas (carbon monoxide and hydrogen) and then via oligomerisation (e.g., the Fischer-Tropsch process) to higher molecular weight molecules that are hydrocracked to produce iso-paraffins in the required lubricant boiling/viscosity range. GTL base stocks are only just being commercialised and consequently there is little or no data relating to them that is freely available. As far as it is known, such GTL base stocks will have viscosity grades similar to poly- $\alpha$ -olefins.

Preferably, the weight ratio of amide to said further base oil will be between 100:0 to 1:99, preferably between 99:1 to 1:99, more preferably between 60:40 and 2:98, more particularly between 40:60 and 3:97, and especially between 20:80 to 5:95.

Preferably, the lubricant composition comprises at least 1 wt % amide, preferably at least 2 wt %, more preferably at least 5 wt % based on the total weight of the composition. Preferably, the lubricant composition comprises up to 99.9 wt % amide, preferably up to 99 wt %, preferably up to 90 wt %, preferably up to 80 wt %, more preferably up to 50 wt %, more particularly up to 30 wt %, most preferably up to 20 wt % and desirably up to 10 wt % based on the total weight of the composition.

As previously described, the lubricant composition may comprise at least 0.1 wt % of said at least one additive, preferably at least 0.5 wt %, more preferably at least 1 wt %, and desirably at least 2 wt % based on the total weight of the composition. The lubricant composition may comprise up to 40 wt % of said at least one additive, preferably up to 30 wt %, more preferably up to 20 wt % and desirably up to 10 wt % based on the total weight of the composition.

Preferably, the lubricant composition comprises at least 1 wt % of a further base oil, preferably at least 20 wt %, more preferably at least 40 wt %, and most preferably at least 60 wt % based on the total weight of the composition. Preferably, the lubricant composition comprises up to 98.9 wt % of a further base oil, preferably up to 98 wt %, more particularly up to 95 wt %, and most preferably up to 90 wt % based on the total weight of the composition.

In one embodiment, the lubricant composition of the present invention is used as an engine oil, preferably an automotive or marine engine oil, more preferably an automotive engine oil. When the lubricant composition is an engine oil, additives are preferably present at a concentration in the range from 0.1 to 30 wt % based on the total weight of the engine oil.

For an automotive engine oil the term further base oil includes both gasoline and diesel (including heavy duty diesel (HDDEO)) engine oils. The further base oil may be chosen from any of the Group I to Group V base oils (which includes Group III+ gas to liquid) or a mixture thereof. Preferably, the further base oil has one of Group II, Group III or a Group IV base oil as its major component, especially Group III. By major component, is meant at least 50%, preferably at least 65%, more preferably at least 75%, especially at least 85% by weight of the further base oil.

The further base oil may also comprise as a minor component, by which is meant preferably less than 30%, more preferably less than 20%, especially less than 10% by weight of co-base oil of any or a mixture of Group III+, IV and/or Group V base oils which have not been used as the major component in the further base oil. Examples of such Group V base oils include alkyl naphthalenes, alkyl aromatics, vegetable oils, esters, for example monoesters, diesters and polyol esters, polycarbonates, silicone oils and polyalkylene glycols. More than one type of Group V base stock may be present. Preferred Group V base stocks are esters, particularly polyol esters.

For an engine oil, the base stock may range from SAE viscosity grade 0 W to 15 W. The viscosity index is preferably at least 90 and more preferably at least 105. The base stock preferably has a viscosity at 100° C. of 3 to 10 mm<sup>2</sup>/s, more preferably 4 to 8 mm<sup>2</sup>/s. The Noack volatility, measured according to ASTM D-5800 is preferably less than 20%, more preferably less than 15%.

Preferably, the engine oil is a low viscosity engine oil, preferably the engine oil has an SAE class rating of less than 5 W, more especially an SAE class rating of 0 W. Low viscosity engine oils are increasingly desirable and a significant proportion of current engine lubricant base oils are not suitable for this purpose. Some disadvantages of such lubricants include the inherent limitation imposed by the viscosity indices of the base oils (which impacts film thickness); and the inability to reduce viscosity without increasing volatility (i.e., increasing the Noack evaporation loss of the lubricant). Additionally, very low viscosity esters can also have high polarity which can lead to seal compatibility issues and potential wear issues due to competition with antiwear agents such as ZDDP when the esters are used at high dose rates, e.g., >15 wt %. For example, di-isoctyl adipate has an NPI of 41. In addition, low viscosity lubricants, which have been optimised to give low volatilities, can also suffer from either low viscosity indices (<125), poor low temperature flow properties or shorter drain intervals resulting from poor oxidative stability (from the use of components in which gem dimethyl branching is present). The amides of the present invention provide a suitable, and in many cases, advantageous alternative to existing engine lubricant base oils for low viscosity systems since they provide good viscosity whilst at the same time providing good hydrolytic, thermal and oxidative stability.

For engine oils, a friction reducing additive may be present at levels of at least 0.2 wt %, preferably at least 0.3 wt %, more preferably at least 0.5 wt % based on the total weight of the engine oil. The friction reducing additive may be present at levels of up to 5 wt %, preferably up to 3 wt %, more preferably up to 2 wt % based on the total weight of the engine oil.

The automotive engine oil may also comprise other types of additives of known functionality at levels between 0.1 to 30 wt %, more preferably between 0.5 to 20 wt %, yet more preferably between 1 to 10 wt % based on the total weight of the engine oil. These further additives can include deter-

## 11

gents, dispersants, oxidation inhibitors, corrosion inhibitors, rust inhibitors, anti-wear additives, foam depressants, pour point depressants, viscosity index improvers and mixtures thereof. Viscosity index improvers may include polyisobutenes, polymethacrylate acid esters, polyacrylate acid esters, diene polymers, polyalkyl styrenes, alkenyl aryl conjugated diene copolymers and polyolefins. Foam depressants may include silicones and organic polymers. Pour point depressants may include polymethacrylates, polyacrylates, polyacrylamides, condensation products of haloparaffin waxes and aromatic compounds, vinyl carboxylate polymers, terpolymers of dialkylfumarates, vinyl esters of fatty acids and alkyl vinyl ethers. Ashless detergents may include carboxylic dispersants, amine dispersants, Mannich dispersants and polymeric dispersants. Antiwear additives may include ZDDP, ashless and ash containing organic phosphorous and organo-sulphur compounds, boron compounds, and organomolybdenum compounds. Ash-containing dispersants may include neutral and basic alkaline earth metal salts of an acidic organic compound. Oxidation inhibitors may include hindered phenols and alkyl diphenylamines. Additives may include more than one functionality in a single additive.

The lubricant composition of the present invention may be used as a gear oil. The gear oil may be an industrial, automotive and/or marine gear oil. When the lubricant composition is a gear oil, additives are preferably present in the range between 0.1 to 30 wt % based on the total weight of the gear oil.

The gear oil may have a kinematic viscosity according to an ISO grade. An ISO grade specifies the mid-point kinematic viscosity of a sample at 40° C. in cSt (mm<sup>2</sup>/s). For example, ISO 100 has a viscosity of 100±10 cSt and ISO 1000 has a viscosity of 1000±100 cSt. The gear oil preferably has a viscosity in the range from ISO 10 to ISO 1500, more preferably ISO 68 to ISO 680.

Gear oils according to the invention preferably have good low temperature properties. For example, the viscosity of such formulations at -35° C. is less than 120,000 centapoise (cP), more preferably less than 100,000 cP, especially less than 90,000 cP.

Industrial gear oils include those suitable for use in gear boxes with spur, helical, bevel, hypoid, planetary and worm gears. Suitable applications include use in mining; mills such as paper, textile and sugar mills; steel production and in wind turbines. One preferred application is in wind turbines where the gear boxes typically have planetary gears.

In a wind turbine, the gear-box is typically placed between the rotor of a wind turbine blade assembly and the rotor of a generator. The gear-box may connect a low-speed shaft turned by the wind turbine blade(s) rotor at about 10 to 30 rotations per minute (rpm), to one or more high speed shafts that drive the generator at about 1000 to 2000 rpm, the rotational speed required by most generators to produce electricity. The high torque exerted in the gear-box can generate huge stress on the gears and bearings in the wind turbine. A gear oil of the present invention may enhance the fatigue life of the gear-box of a wind turbines by reducing the friction between the gears.

Lubricants in wind turbines gearboxes are often subjected to prolonged periods of use between maintenance, i.e. long service intervals. Therefore a long lasting lubricant composition with high stability may be required, so as to provide suitable performance over lengthy durations of time.

Automotive gear oils include those suitable for use in manual transmissions, transfer cases and differentials which all typically use a hypoid gear. By transfer case we mean a

## 12

part of a four wheel drive system found in four wheel drive and all wheel drive systems. It is connected to the transmission and also to the front and rear axles by means of driveshafts. It is also referred to in the literature as a transfer gearcase, transfer gearbox, transfer box or jockey box.

Marine thruster gearboxes have specific gear oils that include a higher proportion of additives, e.g. dispersants, anticorrosives, to deal with corrosion and water entrainment compared to industrial and automotive gear oils. There are also outboard gear oils used for the propeller unit which may be more relevant for smaller vessels.

A gear oil according to the invention may comprise one or more of the additives described herein. The gear oil preferably comprises one or more additive(s) which may include at least one species of extreme-pressure agent selected from the group consisting of sulfur-based additives and phosphorous-based additives, or at least one species of the extreme-pressure agents and at least one species of additive selected from the group consisting of solubilizing agent, friction modifying agent, ashless dispersant, pour point depressant, antifoaming agent, antioxidant, rust inhibitor, and corrosion inhibitor.

Additives may be present in the gear oils of known functionality at levels between 0.01 to 30 wt %, more preferably between 0.01 to 20 wt %, and more especially between 0.01 to 10 wt % based on the total weight of the gear oil. These can include detergents, extreme pressure/antiwear additives, dispersants, corrosion inhibitors, rust inhibitors, friction modifiers, foam depressants, pour point depressants, and mixtures thereof. Extreme pressure/antiwear additives include ZDDP, tricresyl phosphate, amine phosphates. Corrosion inhibitors include sarcosine derivatives, for example CRODASINIC™ O available from Croda Europe Ltd. Foam depressants include silicones and organic polymers. Pour point depressants include polymethacrylates, polyacrylates, polyacrylamides, condensation products of haloparaffin waxes and aromatic compounds, vinyl carboxylate polymers, terpolymers of dialkylfumarates, vinyl esters of fatty acids and alkyl vinyl ethers. Ashless detergents include carboxylic dispersants, amine dispersants, Mannich dispersants and polymeric dispersants. Friction modifiers include amines and partial fatty acid esters of polyhydric alcohols. Ash-containing dispersants include neutral and basic alkaline earth metal salts of an acidic organic compound. Additives may have more than one functionality in a single material.

The gear oil may further comprise an antioxidant preferably in the range 0.2 to 2 wt %, more preferably 0.4 to 1 wt % by weight based on the total weight of the gear oil. Antioxidants include hindered phenols, alkyl diphenylamines and derivatives and phenyl alpha naphthylamines and derivatives thereof. Gear oil compositions with the presence of the antioxidant preferably exhibit a percentage viscosity loss, measured using a modified version of CEC L-40-A-93, over a 100 hour period of less than 20%, more preferably less than 15% and especially less than 10%.

The gear oil preferably comprises at least 0.1 wt %, more preferably at least 0.5 wt %, particularly at least 1 wt %, and especially at least 1.5 wt % of additive(s) (additive pack) based upon the total weight of the gear oil. The gear oil preferably comprises up to 15 wt %, more preferably up to 10 wt %, particularly up to 4 wt %, and especially up to 2.5 wt % of further additive(s) (additive pack) based upon the total weight of the gear oil.

Suitable commercially available additive packs for industrial gear oils include HITEC® 307 (for wind turbines), 315, 317 and 350 (ex Afton); IRGALUBE® ML 605 A (ex

## 13

BASF); LUBRIZOL® IG93MA, 506, 5064 and 5091 (ex Lubrizol); VANLUBE® 0902 (ex Vanderbilt); ADDITIN® RC 9330, ADDITIN® RC 9410 and ADDITIN® RC 9451 (ex Rhein Chemie); NA-LUBE BL-1208 (ex King Industries).

The lubricant composition of the present invention may be used as a hydraulic oil or fluid. When the lubricant composition is a hydraulic oil or fluid, additives are suitably present in the range from 0.1 to 30 wt % based on the total weight of the hydraulic fluid.

The hydraulic fluid may have a viscosity from ISO 10 to ISO 100, preferably from ISO 32 to ISO 68.

Hydraulic fluids find use wherever there is a need to transfer pressure from one point to another in a system. Some of the many commercial applications where hydraulic fluids are utilized are in aircraft, braking systems, compressors, machine tools, presses, draw benches, jacks, elevators, die-castings, plastic moldings, welding, coal-mining, tube reducing machines, paper-machine press rolls, calendar stacks, metal working operations, fork lifts, and automobiles.

A hydraulic oil or fluid according to the invention may comprise one or more of the additives described herein.

The lubricant composition of the present invention may be used as a metalworking fluid. When the lubricant composition is a metal working fluid, additives are preferably present in the range between 1 to 40 wt % based on the total weight of the metal working fluid.

The metal working fluid may have a viscosity of at least ISO 10, preferably at least ISO 100.

Metalworking operations include for example, rolling, forging, hot-pressing, blanking, bending, stamping, drawing, cutting, punching, spinning and the like and generally employ a lubricant to facilitate the operation. Metalworking fluids generally improve these operations in that they can provide films of controlled friction or slip between interacting metal surfaces and thereby reduce the overall power required for the operations, and prevent sticking and decrease wear of dies, cutting bits and the like. Sometimes the lubricant is expected to help transfer heat away from a particular metalworking contact point.

Metal working fluids often comprise a carrier fluid and one or more additives. The carrier fluid imparts some general lubricity to the metal surface and carries/delivers the specialty additives to the metal surfaces. Additionally, the metal working fluid may provide a residual film on the metal part thereby adding a desired property to the metal being processed. The additives can impart a variety of properties including friction reduction beyond hydrodynamic film lubrication, metal corrosion protection, extreme pressure or anti-wear effects. The carrier fluid may be a further base oil as described herein.

Carrier fluids include various petroleum distillates including American Petroleum Institute Group I to V base stocks. The additives can exist within the carrier fluid in a variety of forms including as dissolved, dispersed in, and partially soluble materials. Some of the metal working fluid may be lost to or deposited on the metal surface during the working process; or may be lost to the environment as spillage, sprays, etc., and may be recyclable if the carrier fluid and additives have not degraded significantly during use. Due to entry of a percentage of the metal working fluid into process goods and industrial process streams, it is desirable if the components to the metal working fluid are eventually biodegradable and pose little risk of bioaccumulation to the environment.

## 14

The metalworking fluid may comprise up to 90 wt % in total of amide plus further base oil, more preferably up to 80 wt % based on the total weight of the metal working fluid.

A metalworking fluid according to the invention may comprise one or more of the additives described herein. The metalworking fluid may comprise at least 10 wt % of additives based on the total weight of the metal working fluid.

The lubricant composition of the present invention may be used as a refrigerant oil. When the lubricant composition is a refrigerant oil, one or more additives are preferably present in the range between 1 to 20 wt % based on the total weight of the refrigerant oil.

The refrigerant oil may have a viscosity of from ISO 10 to ISO 500, preferably ISO 20 to ISO 250.

Refrigerant oils are used in compressor systems where lubrication is required, in particular since heat generation in moving parts due to friction must be minimised. A refrigerant oil according to the present invention may comprise one or more of the additives described herein. A refrigerant oil may also comprise a further base oil of the type described above. Preferably, when present, the further base oil is a polyol ester base oil (POE oil).

Any of the above features may be taken in any combination and with any aspect of the invention.

## EXAMPLES

The present invention will now be described further, for illustrative purposes only, in the following examples. All parts and percentages are given by weight, based on the total weight of the material or composition as appropriate, unless otherwise stated.

## 35 Synthesis Examples

## Example 1

To a 1 liter round bottom flask equipped with Dean-Stark apparatus connected with water condenser was charged isostearic acid (284 g, 1 mol), (Di-2-ethylhexyl)amine (295 g, 1.05 mol) and sodium hypophosphite (3 g, 0.028 mol). The reaction mixture was heated from room temperature to 240° C. over 40 minutes. The water was generated from the reaction and collected/separated in the Dean-Stark. Organics were refluxed from Dean-Stark to the flask. Reaction was held at 240° C. until the acid value was below 1.0. The vacuum was gradually applied at 250-200 mmHg for 1 hour, then followed by stripping of excess (di-2-ethylhexyl)amine at 35 mmHg/240° C. until base number was below 2. The reaction mixture was cooled at 110° C., filtered through a filter paper under full vacuum to give the product as clear liquid, straw color. The sample was taken for QC analysis which generated the results below.

40 <sup>1</sup>H NMR (400 MHz, CDCl<sub>3</sub>) δ 3.40-3.20 (2H, m), 3.20-3.05 (2H, m), 2.40-2.20 (2H, m), 1.90-1.50 (4H, m), 1.50-1.10 (41H, m), 1.10-0.60 (18H, m)

45 <sup>13</sup>C NMR (100 MHz, CDCl<sub>3</sub>) δ 173.4, 51.3, 48.7, 38.7, 37.0, 36.9, 33.4, 32.7, 32.4, 32.2, 30.0-29.0 multiple peaks, 29.0-28.3 multiple peaks, 27.2-26.5 multiple peaks, 25.6, 23.9, 23.8, 23.0, 22.9, 22.6, 19.6 multiple peaks, 14.5-14.5 multiple peaks, 11.0-10.2 multiple peaks.

## Example 2

To a 1 liter round bottom flask equipped with Dean-Stark apparatus connected with water condenser was charged

**15**

2-Ethylhexanoic acid (184 g, 1.2 mol), (Di-2-ethylhexyl)amine (281 g, 1 mol) and sodium hypophosphite (3 g, 0.028 mol). The reaction mixture was heated from room temperature to 240° C. over 40 minutes. The water was generated from the reaction and collected/separated in the Dean-Stark. Organics were refluxed from Dean-Stark to the flask. Reaction was held at 240° C. until the acid value was below 1.0. The vacuum was gradually applied at 250-200 mmHg for 1 hour, then followed by stripping of excess 2-ethylhexanoic acid at 35 mmHg/240° C. until AV was below 1. The reaction mixture was cooled at 110° C., filtered through a filter paper under full vacuum to give the product as liquid amide. The sample was taken for QC analysis which generated the results below.

<sup>1</sup>H NMR (400 MHz, CDCl<sub>3</sub>) δ 3.40-3.10 (4H, m), 2.60-2.40 (1H, m), 1.85-1.55 (4H, m), 1.55-1.40 (2H, m), 1.40-1.15 (20H, m), 1.05-0.75 (18H, m)

<sup>13</sup>C NMR (100 MHz, CDCl<sub>3</sub>) δ 176.2, 51.9, 51.8, 50.2-49.6 multiple peaks, 42.8, 39.3, 39.2, 37.2, 32.3, 32.2, 30.5, 29.8-29.7 multiple peaks, 28.0-27.4 multiple peaks, 25.7, 23.6, 23.5, 22.9, 22.8, 13.9, 13.8, 12.0, 10.7, 10.4.

## Example 3

To a 1 liter round bottom flask equipped with Dean-Stark apparatus connected with water condenser was charged Adipic Acid (146 g, 1.0 mol), (Di-2-ethylhexyl)amine (600 g, 2.1 mol) and sodium hypophosphite (3 g, 0.028 mol). The reaction mixture was heated from room temperature to 240° C. over 40 minutes. The water was generated from the reaction and collected/separated in the Dean-Stark. Organics were refluxed from Dean-Stark to the flask. Reaction was held at 240° C. until the acid value was below 1.0. The vacuum was gradually applied at 250-200 mmHg for 1 hour, then followed by stripping of excess Di-(2-ethylhexyl)amine at 35 mmHg/240° C. until base number was below 0.5. The reaction mixture was cooled at 110° C., filtered through a filter paper under full vacuum to give the product as liquid amide. The sample was taken for QC analysis which generated the results below.

<sup>1</sup>H NMR (400 MHz, CDCl<sub>3</sub>) δ 3.40-3.20 (4H, m), 3.20-3.10 (4H, m), 2.45-2.25 (4H, m), 1.80-1.65 (6H, m), 1.65-1.50 (2H, m), 1.45-1.10 (32H, m), 1.05-0.75 (24H, m)

<sup>13</sup>C NMR (100 MHz, CDCl<sub>3</sub>) δ 172.6, 51.1, 49.4, 38.2, 36.7, 30.2, 30.1, 28.2, 28.1, 25.0, 23.6, 23.5, 23.4, 22.7, 22.6, 13.6, 10.5, 10.2

## Example 4

To a 1 liter round bottom flask equipped with Dean-Stark apparatus connected with water condenser was charged 3,5,5'-trimethylhexanoic acid (284 g, 1.9 mol), (Di-2-ethylhexyl)amine (295 g, 1.05 mol) and sodium hypophosphite (3 g, 0.028 mol). The reaction mixture was heated from room temperature to 240° C. over 40 minutes. The water was generated from the reaction and collected/separated in the Dean-Stark. Organics were refluxed from Dean-Stark to the flask. Reaction was held at 240° C. until the acid value was below 1.0. The vacuum was gradually applied at 250-200 mmHg for 1 hour, then followed by stripping of excess Di-(2-ethylhexyl)amine at 35 mmHg/240° C. until base number was below 2. The reaction mixture was cooled at 110° C., filtered through a filter paper under full vacuum to give the product as liquid amide. The sample was taken for QC analysis which generated the results below.

**16**

<sup>1</sup>H NMR (400 MHz, CDCl<sub>3</sub>) δ 3.45-3.25 (2H, m), 3.25-3.10 (2H, m), 2.40-2.20 (3H, m), 1.56-1.53 (1H, m), 1.53-1.51 (1H, m), 1.50-1.15 (18H, m), 1.10-0.70 (24H, m)

<sup>13</sup>C NMR (100 MHz, CDCl<sub>3</sub>) δ 172.5, 51.5, 51.0, 48.9, 43.0, 38.5, 36.9, 31.0, 30.7-30.2 multiple peaks, 30.1, 30.0, 28.6, 28.5, 27.0, 23.7, 23.6, 23.5, 22.9, 22.8, 22.7, 22.4, 14.0, 14.9, 10.8, 10.7, 10.5

## Example 5

To a 1 liter round bottom flask equipped with Dean-Stark apparatus connected with water condenser was charged C8-10 fatty acid (C-810L supplied by P&G) (200 g, 1.31 mol), (Di-2-ethylhexyl)amine (281 g, 1 mol) and sodium hypophosphite (3 g, 0.028 mol). The reaction mixture was heated from room temperature to 240° C. over 40 minutes. The water was generated from the reaction and collected/separated in the Dean-Stark. Organics were refluxed from Dean-Stark to the flask. Reaction was held at 240° C. until the acid value was below 1.0. The vacuum was gradually applied at 250-200 mmHg for 1 hour, then followed by stripping of excess acid at 35 mmHg/240° C. until AV was below 0.5. The reaction mixture was cooled at 110° C., filtered through a filter paper under full vacuum to give the product as liquid amide.

## Example 6

To a 1 liter round bottom flask equipped with Dean-Stark apparatus connected with water condenser was charged Lauric Acid (210 g, 1.05 mol), (Di-2-ethylhexyl)amine (337 g, 1.20 mol) and sodium hypophosphite (3 g, 0.028 mol). The reaction mixture was heated from room temperature to 240° C. over 40 minutes. The water was generated from the reaction and collected/separated in the Dean-Stark. Organics were refluxed from Dean-Stark to the flask. Reaction was held at 240° C. until the acid value was below 1.0. The vacuum was gradually applied at 250-200 mmHg for 1 hour, then followed by stripping of excess Di-(2-ethylhexyl)amine at 35 mmHg/240° C. until base number was below 2. The reaction mixture was cooled at 110° C., filtered through a filter paper under full vacuum to give the product as liquid amide.

## Example 6A

To a 1 liter round bottom flask equipped with Dean-Stark apparatus connected with water condenser was charged pre-melted coconut fatty acid (250 g with major fatty acid components including C12/lauric at about 50 wt % and C14/myristic at about 18 wt %), di-(2-ethylhexyl)-amine (358 g), and sodium hypophosphite (3 g). The reaction mixture was heated from room temperature to 240° C. over 2 hours. The water was generated from the reaction and collected/separated in the Dean-Stark. Organics were refluxed from Dean-Stark to the flask. Reaction was held at 240° C. until the acid value was below 0.5. Vacuum was gradually applied at 100 mmHg to strip excess Di-(2-ethylhexyl)amine until the alkali value was below 0.5. The reaction mixture was cooled at 80° C., filtered through a filter paper under full vacuum to give the product as liquid amide.

## Example 7

To a 1 liter round bottom flask equipped with Dean-Stark apparatus connected with water condenser was charged

## 17

2-Ethylhexanoic acid (288 g, 2 mol), diisopropylamine (240 g, 2.4 mol), and sodium hypophosphite (3 g, 0.028 mol). The reaction mixture was heated from room temperature to 220° C. over 180 minutes. The water was generated from the reaction and collected/separated in the Dean-Stark. Organics were refluxed from Dean-Stark to the flask. Reaction was held at 220° C. until the acid value was below 1.0. The vacuum was gradually applied at 250-200 mmHg for 1 hour, then followed by stripping of excess amine at 35 mmHg/240° C. until base number was below 2. The reaction mixture was cooled at 110° C., filtered through a filter paper under full vacuum to give the product as liquid amide. The sample was taken for QC analysis which generated the results below.

<sup>1</sup>H NMR (400 MHz, CDCl<sub>3</sub>) 4.50-4.20 (1H, m), 3.55-<sup>15</sup> 3.35 (1H, m), 2.6-2.45 (1H, m), 1.75-1.16 (2H, m), 1.5-1.2 (6H, m), 1.47 (6H, d, J=6.78 Hz), 1.21 (6H, d, J=6.78 Hz), 0.95-0.80 (6H, m)

<sup>13</sup>C NMR (100 MHz, CDCl<sub>3</sub>) 174.3, 47.7, 45.8, 43.4, 32.6, 29.5, 25.9, 22.6, 20.6, 20.4, 13.6, 11.7

## Example 8

To a 1 liter round bottom flask equipped with Dean-Stark apparatus connected with water condenser was charged Isostearic acid (288 g, 1 mol), diisopropyl amine (280 g, 2.17 mol) and sodium hypophosphite (3 g, 0.028 mol). The reaction mixture was heated from room temperature to 220° C. over 40 minutes. The water was generated from the reaction and collected/separated in the Dean-Stark. Organics were refluxed from Dean-Stark to the flask. Reaction was held at 220° C. until the acid value was below 1.0. The vacuum was gradually applied at 250-200 mmHg for 1 hour, then followed by stripping of excess amine at 35 mmHg/240° C. until base number was below 2. The reaction mixture was cooled at 110° C., filtered through a filter paper under full vacuum to give the product as liquid amide.

## Example 9

To a 1 liter round bottom flask equipped with Dean-Stark apparatus connected with water condenser was charged

stearic acid (249 g, 0.876 mol), (Di-2-ethylhexyl)amine (259 g, 0.92 mol) and sodium hypophosphite (3 g, 0.028 mol). The reaction mixture was heated from room temperature to 240° C. over 40 minutes. The water was generated from the reaction and collected/separated in the Dean-Stark. Organics were refluxed from Dean-Stark to the flask. Reaction was held at 240° C. until the acid value was below 1.0. The vacuum was gradually applied at 250-200 mmHg for 1 hour, then followed by stripping of excess Di-(2-ethylhexyl)amine at 35 mmHg/240° C. until base number was below 2. The reaction mixture was cooled at 110° C., filtered through a filter paper under full vacuum to give the product as liquid amide.

## Examples 10 to 13

The method set out above for the production of Examples 1 to 9 was followed with the reactants set out in Table 1 below to produce further amides.

TABLE 1

| Example | Amine                                | Acid                 |
|---------|--------------------------------------|----------------------|
| 10      | Diisobutylamine                      | 2-ethylhexanoic acid |
| 11      | Ditridecylamine (mixture of isomers) | 2-ethylhexanoic acid |
| 12      | Di-(2-ethylhexyl)amine               | C36 dimer acid       |
| 13      | Di-(2-ethylhexyl)amine               | Sebacic acid         |

## Properties of Examples 1 to 10

The physical properties of the amides produced in Examples 1 to 10 above were measured according to industry standard methods, and the results are recorded in Table 2 below. The properties of four well-known lubricant base oils have also been included in the table by way of comparison.

TABLE 2

| Example                                               | Kinetic Viscosity @40° C. | Kinetic Viscosity @100° C. | Acid Value (mg KOH/g) | Alkali Number (mg KOH/g) | Pour Point (° C.) |
|-------------------------------------------------------|---------------------------|----------------------------|-----------------------|--------------------------|-------------------|
| 1                                                     | 58                        | 7.6                        | 0.18                  | 0.3                      | -42               |
| 2                                                     | 26.5                      | 3.85                       | 0.7                   | 0.15                     | -49               |
| 3                                                     | 199                       | 13.7                       | 0.35                  | 0.17                     | -21               |
| 4                                                     | 30.15                     | 4.21                       | 3.89                  | 0.15                     | -39               |
| 5                                                     | 19.6                      | 3.6                        | 0.21                  | 0.36                     | -55               |
| 6                                                     | 40.5                      | 5.0                        | 0.12                  | 1.05                     | -39               |
| 7                                                     | 7.1                       | 2.0                        | 0.56                  | 0.43                     | -55               |
| 8                                                     | 8.7                       | 2.5                        | 0.4                   | 0.67                     | -55               |
| 9                                                     | 37.42                     | 6.27                       | 1.5                   | 1.94                     | -22               |
| 10                                                    | 7.6                       | 2.2                        |                       |                          | ≤-60              |
| Comparative A: Monoester (PRIOLUBE™ 1415, ex Croda)   | 8.5                       | 2.7                        | 0.2                   |                          | -27               |
| Comparative B: Diester (PRIOLUBE™ 1936, ex Croda)     | 26                        | 5.3                        | 0.05                  |                          | -54               |
| Comparative C: Polyolester (PRIOLUBE™ 3970, ex Croda) | 20                        | 4.4                        | 0.05                  |                          | -51               |
| Comparative D: Polyolester (PRIOLUBE™ 1976, ex Croda) | 320                       | 23                         | 0.5                   |                          | -27               |

## Performance Examples

## Example 14

## Hydrolytic Stability Evaluation

To evaluate hydrolytic stability two ASTM test methods were used: ASTM D2619—Standard Test Method for Hydrolytic Stability of Hydraulic Fluids (Beverage Bottle Method), and ASTM D943 Standard Test Method for Oxidation Characteristics of Inhibited Mineral Oils, which is also reflective of hydrolytic stability of lubricants.

ASTM D943 Standard Test Method for Oxidation Characteristics of Inhibited Mineral Oils was originally used for determination of oxidative stability of mineral oils, however later it was determined that it can also be used to evaluate hydrolytic stability of ester-based lubricants. Oils exposed to atmospheric oxygen may form sludge and carboxylic acids in a reaction catalyzed by water and metals.

In this example, 300 ml of the test material and 60 ml water were heated together in a test tube with an iron-copper catalyst to 95° C. Oxygen was bubbled through the test material-water mixture at a controlled rate. Periodically, usually at hourly intervals, a small aliquot of oil was removed and the acid number determined. The test was deemed to have finished, and the number of hours from the start of the test recorded, when the acid number reached 2 mg KOH.

In this example, results from the evaluation of hydrolytic stability of the neat amides of Examples 1 and 2 were compared against esters commonly used in lubricant applications. In particular, Comparative A (2-Ethylhexyl Oleate, available from Croda under PRIOLUBE™ 1415), Comparative B (Triisodecyladipate, available from Croda under PRIOLUBE™ 1936), Comparative C (TMP caprate/caprylate, available from Croda under PRIOLUBE™ 3970), and Comparative D (Pentaerythritol tetra-3,5,5-trimethylhexanoate, ester with exceptional oxidative and hydrolytic stability available from Croda under PRIOLUBE™ 1965) were compared with the amides of Examples 1 and 2. The results are shown in Table 3 below.

TABLE 3

| Hydrolytic and oxidative stability of neat materials |                         |
|------------------------------------------------------|-------------------------|
| Test material                                        | ASTM D943 result, hours |
| Comparative A                                        | 8                       |
| Comparative B                                        | 13                      |
| Comparative C                                        | 36                      |
| Comparative D                                        | 23                      |
| Example 1                                            | 52                      |
| Example 2                                            | 672*                    |

\*Test still on-going at time of reporting, with current acid number 0.96 mg KOH

ASTM D2619 determines the ability of a lubricant composition to resist hydrolysis. Compositions which are unstable to water under the conditions of the test form corrosive acidic and insoluble contaminants.

75 g of the lubricant composition to be tested, 25 g of water, and a polished copper strip were sealed in a bottle then placed in a 200° F. (93° C.) oven and rotated end for end at 5 rpm for 48 hrs. The values reported for each composition at the end of the test were Acid Number Change, Total Acidity of Water, Weight Change and Appearance of Copper Strip. The results are shown in Table 4 below.

In this example, the lubricant compositions used to evaluate hydrolytic stability were based on a standard gear oil and were formulated as follows:

- 10 10% mass of test material  
5 87.35% mass of GR IV basestock (PAO)  
2.65% mass of HITEC® 307 gear oil additive (Afton Chemical)

TABLE 4

| Test material,<br>10% in gear oil<br>formulation | Change in Acid<br>Number (ASTM<br>D974, Organic<br>layer, mg KOH) | Total<br>Acidity<br>of Water<br>Layer (mg<br>KOH) | Weight<br>Change of<br>Copper<br>Panel   |                                  | Appearance<br>of Copper<br>Panel |
|--------------------------------------------------|-------------------------------------------------------------------|---------------------------------------------------|------------------------------------------|----------------------------------|----------------------------------|
|                                                  |                                                                   |                                                   | Copper<br>Panel<br>(mg/cm <sup>3</sup> ) | Appearance<br>of Copper<br>Panel |                                  |
| Comparative A                                    | 1.81                                                              | 25.93                                             | 0.000                                    | Shiny 1B-2A                      |                                  |
| Comparative B                                    | 1.41                                                              | 25.96                                             | -0.375                                   | Shiny 1B                         |                                  |
| Comparative C                                    | 0.63                                                              | 15.75                                             | -0.058                                   | Shiny 1B-2A                      |                                  |
| Comparative D                                    | 0.61                                                              | 15.97                                             | -0.042                                   | Dull 4A                          |                                  |
| Example 1                                        | -0.27                                                             | 15.75                                             | -0.033                                   | Shiny 1B-2A                      |                                  |
| Example 2                                        | -0.2                                                              | 12.50                                             | 0.017                                    | Shiny 3A                         |                                  |

## Example 15

## Volatility Evaluation

The volatility of the neat test materials was measured 30 according to test method ASTM D6375-09 Standard Test Method for Evaporation Loss of Lubricating Oils by Thermogravimetric Analyzer (TGA) Noack Method. Comparative Examples E (GRII Mineral oil (PURE PERFORMANCE® 110N, from Phillips 66 Co)) and F (PAO4 35 (SPECTRASYN™ 4, Exxon Chemicals)) were added to the test matrix for comparison. The results are shown in Table 5 below.

TABLE 5

| Test Material | ASTM D6375 (NOACK) |             |
|---------------|--------------------|-------------|
|               | weight loss, wt %  | KV 100, cSt |
| Comparative A | 30                 | 2.7         |
| Comparative B | 12                 | 5.3         |
| Comparative C | 2.45               | 4.4         |
| Comparative D | 1.70               | 23          |
| Example 1     | 15.0               | 7.6         |
| Example 2     | 57.8               | 3.85        |
| Example 3     | 3.2                | 13.7        |
| Comparative E | 26.5               | 4.2         |
| Comparative F | 14.0               | 4.0         |

## Example 16

## Solubility of Additives

The relative solubilities of various lubricant additives 60 were tested by blending the respective additives and additive packages into PAO 40 (SPECTRASYN™ 40, available from ExxonMobil Chemicals) along with a second base oil selected from the amides of Examples 1 and 2, esters of Comparatives B and C or PAO 4 (SPECTRASYN™ 4, available from ExxonMobil Chemicals). The blending was 65 facilitated by stirring the lubricant base oils (PAO 40 and second base oil) and the additive, or additive package, at 65°

C. for 1 hour with 600 RPM agitation. After blending was complete, the resulting oil samples were sealed in air-tight jars and stored for 30 days at 24° C. After once month (30 days) of storage, the lubricant samples were inspected visually and the appearances were recorded. The results are shown below in Tables 6, 7 and 8.

The additives tested were Glycerol Monooleate (GMO, available from Croda Inc as PRIOLUBE™ 1407), Molybdenum dialkyldithiocarbamate (MOLYVAN® 822, available from Vanderbilt Chemicals LLC), and an industrial gear oil package (HITEC® 307, available from Afton Chemical Corporation).

TABLE 6

| Blends containing 1 wt % of Glycerol Monooleate (all numbers are wt %) |               |               |           |           |       |                          |
|------------------------------------------------------------------------|---------------|---------------|-----------|-----------|-------|--------------------------|
| PAO 4                                                                  | Comparative B | Comparative C | Example 1 | Example 2 | PAO40 | Solubility test results. |
| 10                                                                     |               |               |           |           | 89    | Sediment                 |
|                                                                        | 10            |               |           |           | 89    | Slight haze              |
|                                                                        |               | 10            |           |           | 89    | Slight haze              |
|                                                                        |               |               | 10        |           | 89    | Clear                    |
|                                                                        |               |               |           | 10        | 89    | Clear                    |
| 5                                                                      |               |               |           |           | 94    | Sediment                 |
|                                                                        | 5             |               |           |           | 94    | Sediment                 |
|                                                                        |               | 5             |           |           | 94    | Sediment                 |
|                                                                        |               |               | 5         |           | 94    | Clear                    |
|                                                                        |               |               |           | 5         | 94    | Clear                    |

TABLE 7

| Blends containing 1 wt % of Molybdenum dialkyldithiocarbamate (all numbers are wt %) |               |               |           |           |       |                          |
|--------------------------------------------------------------------------------------|---------------|---------------|-----------|-----------|-------|--------------------------|
| PAO 4                                                                                | Comparative B | Comparative C | Example 1 | Example 2 | PAO40 | Solubility test results. |
| 10                                                                                   |               |               |           |           | 89    | Sediment                 |
|                                                                                      | 10            |               |           |           | 89    | Slight haze              |
|                                                                                      |               | 10            |           |           | 89    | Slight haze              |
|                                                                                      |               |               | 10        |           | 89    | Clear                    |
|                                                                                      |               |               |           | 10        | 89    | Clear                    |
| 5                                                                                    |               |               |           |           | 94    | Sediment                 |
|                                                                                      | 5             |               |           |           | 94    | Sediment                 |
|                                                                                      |               | 5             |           |           | 94    | Slight Haze              |
|                                                                                      |               |               | 5         |           | 94    | Clear                    |
|                                                                                      |               |               |           | 5         | 94    | Clear                    |

TABLE 8

| Blends containing 2.65 wt % of HITEC® 307 gear oil additive (all numbers are wt %) |               |               |           |           |       |                          |
|------------------------------------------------------------------------------------|---------------|---------------|-----------|-----------|-------|--------------------------|
| PAO 4                                                                              | Comparative B | Comparative C | Example 1 | Example 2 | PAO40 | Solubility test results. |
| 10                                                                                 |               |               |           |           | 87.35 | Separation               |
|                                                                                    | 10            |               |           |           | 87.35 | Slight haze              |
|                                                                                    |               | 10            |           |           | 87.35 | Clear                    |
|                                                                                    |               |               | 10        |           | 87.35 | Clear                    |
|                                                                                    |               |               |           | 10        | 87.35 | Clear                    |
| 5                                                                                  |               |               |           |           | 92.35 | Separation               |
|                                                                                    | 5             |               |           |           | 92.35 | Haze                     |
|                                                                                    |               | 5             |           |           | 92.35 | Slight Haze              |
|                                                                                    |               |               | 5         |           | 92.35 | Clear                    |
|                                                                                    |               |               |           | 5         | 92.35 | Clear                    |

As described and shown by way of example above, the lubricant composition and amide, which is the reaction product of a secondary, branched amine and a carboxylic acid, of the present invention provide a commercially viable

and enhanced alternative when compared to existing lubricant materials and compositions.

Any or all of the disclosed features, and/or any or all of the steps of any method or process described, may be combined in any combination.

Each feature disclosed herein may be replaced by alternative features serving the same, equivalent or similar purpose. Therefore, each feature disclosed is one example only of a generic series of equivalent or similar features.

The above statements apply unless expressly stated otherwise. The term specification, for these purposes, includes the description and any accompanying claims, abstract and drawings.

The invention claimed is:

1. A lubricating composition comprising:

a) 5 wt % to 20 wt % based on the total weight of the composition of an amide, where the amide is a liquid at room temperature, has a pour point measured according to the method set out in ASTM D97 of not higher than -20° C. and is of Formula (Ia) or (Ib)



wherein:

R<sup>1</sup> and R<sup>2</sup> are independently selected from the group consisting of an isopropyl group and a C<sub>3</sub> to C<sub>18</sub> branched, saturated or unsaturated, hydrocarbyl group;

R<sup>3</sup> is selected from the group consisting of C<sub>3</sub> to C<sub>23</sub> linear or branched, saturated or unsaturated hydrocarbyl groups;

R<sup>4</sup> is selected from the group consisting of C<sub>1</sub> to C<sub>12</sub> linear or branched, saturated or unsaturated hydrocarbylene groups; and

n is 0 or 1;

b) 0.5 wt % to 2 wt % based on the total weight of the composition of at least one additive that is a molybdenum dialkyldithiocarbamate; and

c) 40 wt % to 95 wt % based on the total weight of the composition of a base oil comprising a lubricant component selected from API Groups IV, IV+ and mixtures of IV or IV+ with one or more of API Groups I, II, III, III+ and V, wherein for the mixtures, the Group IV or IV+ component is the majority component.

2. The lubricant composition according to claim 1, wherein the amide is of Formula (1a).

3. The lubricant composition according to claim 2, wherein R<sup>3</sup> is a C<sub>5</sub> to C<sub>21</sub> alkyl or alkenyl group.

4. The lubricant composition according to claim 1, wherein the amide is of Formula (1b).

5. The lubricant composition according to claim 4, wherein R<sup>4</sup> is a C<sub>1</sub> to C<sub>8</sub> alkylene or alkenylene group.

6. The lubricant composition according to claim 1, wherein the amide of Formula (1a) or Formula (1b) has a hydrolytic stability measured according to the method set out in ASTM D943 of at least 40 hours.

23

7. A method of increasing the additive solubility or detergency of a lubricant composition which comprises adding to the lubricant composition:

a) 5 wt % to 20 wt % based on the total weight of the composition of an amide, where the amide is a liquid at room temperature, has a pour point measured according to the method set out in ASTM D97 of not higher than -20° C. and is of Formula (Ia) or (Ib)



wherein:

R<sup>1</sup> and R<sup>2</sup> are independently selected from the group consisting of an isopropyl group and a C<sub>3</sub> to C<sub>18</sub> branched, saturated or unsaturated, primary hydrocarbyl group;

R<sup>3</sup> is selected from the group consisting of C<sub>3</sub> to C<sub>23</sub> linear or branched, saturated or unsaturated hydrocarbyl groups;

R<sup>4</sup> is selected from the group consisting of C<sub>1</sub> to C<sub>12</sub> linear or branched, saturated or unsaturated hydrocarbylene groups; and

n is 0 or 1; and

b) 0.5 wt % to 2 wt % based on the total weight of the composition of at least one additive that is a molybdenum dialkyldithiocarbamate,

wherein the lubricant composition comprises 40 wt % to 95 wt % based on the total weight of the composition of a base oil comprising a lubricant component selected from API Groups IV, IV+ and mixtures of IV or IV+ with one or more of API Groups I, II, III, III+ and V, wherein for the mixtures, the Group IV or IV+ component is the majority component.

8. A method of producing a hydrolytically stable lubricant composition comprising:

a) reacting a secondary, branched amine and a carboxylic acid to form an amide; and

b) adding at least one additive that is a molybdenum dialkyldithiocarbamate to the amide,

wherein the secondary, branched amine reactant has the formula (II):



24

wherein R<sup>1</sup> and R<sup>2</sup> are independently selected from the group consisting of an isopropyl group, and a C<sub>3</sub> to C<sub>18</sub> branched, saturated or unsaturated, hydrocarbyl group, and

wherein the amide is a liquid at room temperature, has a pour point measured according to the method set out in ASTM D97 of not higher than -20° C. and is of Formula (Ia) or (Ib):



wherein:

R<sup>1</sup> and R<sup>2</sup> are as defined;

R<sup>3</sup> is selected from the group consisting of C<sub>3</sub> to C<sub>23</sub> linear or branched, saturated or unsaturated hydrocarbyl groups;

R<sup>4</sup> is selected from the group consisting of C<sub>1</sub> to C<sub>12</sub> linear or branched, saturated or unsaturated hydrocarbylene groups; and

n is 0 or 1, and

wherein:

the amide is present in the lubricant composition in an amount of 5 wt % to 20 wt % based on the total weight of the composition,

the additive is present in the lubricant composition in an amount of 0.5 wt % to 2 wt % based on the total weight of the composition, and

the lubricant composition comprises 40 wt % to 95 wt % based on the total weight of the composition of a base oil comprising a lubricant component selected from API Groups IV, IV+ and mixtures of IV or IV+ with one or more of API Groups I, II, III, III+ and V, wherein for the mixtures, the Group IV or IV+ component is the majority component.

9. The lubricating composition according to claim 1, wherein the C<sub>3</sub> to C<sub>18</sub> branched, saturated or unsaturated, hydrocarbyl group of R<sup>1</sup> and R<sup>2</sup> is selected from di-(2-ethylhexyl)amine, diisopropylamine, isomers of diti-decylamine, and diisobutylamine.

10. The lubricating composition according to claim 1, wherein the base oil further comprises a mineral oil.

11. The lubricating composition according to claim 1, wherein the base oil comprises a poly- $\alpha$ -olefin derived from C<sub>8</sub> to C<sub>12</sub>  $\alpha$ -olefins and having a kinematic viscosity in the range 3.6 cSt to 8 cSt at 100° C.

12. The lubricating composition according to claim 1, wherein the base oil further comprises at least one of alkyl naphthalenes and alkyl benzenes and esters.

13. The lubricating composition according to claim 1, wherein the base oil further comprises a GTL base stock.

\* \* \* \* \*